

May 19, 1959

T. W. VAN RIJSSEL ET AL

2,887,595

TELEVISION CAMERA TUBE

Filed May 10, 1956



INVENTOR

TIJS WILLEM VAN RIJSSEL  
MARTINUS WILLIBALDUS AUGUSTINUS BOERS  
JOHANNES HENDRICUS JOSEPHUS MAARTENS  
JAN RIGTE BOERMAN  
BY WALTER HEINRICH KÜHL

*Walter Heinrich Kühl*

AGENT

## 1

2,887,595

## TELEVISION CAMERA TUBE

Tijs Willem van Rijssel, Martinus Willibaldus Augustinus Boers, Johannes Hendricus Josephus Maartens, Jan Rigte Boerman, and Walter Heinrich Kuhl, all of Eindhoven, Netherlands, assignors, by mesne assignments, to North American Philips Company, Inc., New York, N.Y., a corporation of Delaware

Application May 10, 1956, Serial No. 583,970

Claims priority, application Netherlands May 14, 1955

9 Claims. (Cl. 313—65)

The invention relates to a television camera tube of the kind in which a charge pattern is produced by secondary emission. The tube comprises a photo-electric cathode. Electrons set free from this cathode by projecting a luminous image onto it are accelerated in the tube and focused onto an image electrode, where they produce secondary emission, owing to which a charge pattern corresponding to the luminous image is produced on the side of the image electrode facing the photo-electric cathode (image side).

It is known that the image electrode of such a camera tube may be made of a substance which permits an electric charge to leak from one side of the electrode to the other. The specific resistance of this substance should be within the range from  $10^9$  to  $10^{12}$  ohm-cm. To this end so-called conductive glass is particularly suitable, an example being the glass known in the United States of America as G—B glass, exhibiting a specific resistance of about  $5 \times 10^{10}$  ohm-cm.

It is advantageous to have a high secondary-emission coefficient on the surface of the image electrode on the image side. It has therefore been suggested to provide the image electrode on the image side with a thin layer of an alkali oxide or alkaline earth oxide to increase this coefficient. However, it has been found that the improvement obtained by such an oxide layer on conductive glass is not always persistent and that in some of the known tubes the increase in efficiency obtained by secondary emission gradually falls off.

This phenomenon becomes manifest with an increase in the collector accelerating voltage, i.e. the voltage at which the secondary electrons are conducted away as completely as possible to the collector. The invention provides means to obviate this disadvantage and to obtain a higher efficiency and longer lifetime of the tube.

In a television camera tube according to the invention, which tube comprises cesium and is provided with an image electrode of conductive glass, on which secondary emission produced by electrons emanating from a photo-electric cathode produces a charge pattern corresponding to a luminous image projected onto the photo-electric cathode and which is provided on the image side with a thin secondary-emissive layer (referred to herein-after as the coating), this layer consists mainly of an inorganic sodium or lithium-halogen compound.

It is known that layers of an oxide or a halogenide of an alkali-, an alkaline-earth- or an earth metal on a metal electrode exhibit a comparatively strong emission.

It is furthermore known that the insulating image electrode of a camera tube operating with an electron beam focused on this electrode, where it sets free secondary electrons, may be constituted by an insulating layer of chloride or bromide of one or more alkali metals, for example KCl or NaCl, which is applied to a metal electrode. If necessary, an insulating layer for example of mica may be sandwiched between the said layer and the metal electrode.

## 2

A camera tube has furthermore been described, of which the image electrode is constituted by a thin insulating or semi-conductive layer, which may be made of an alkali halogenide and which is metal-coated on the rear side. This image electrode is scanned on the metal-coated side by rapid electrons which must render the image electrode conductive.

In none of these known cases, in which reference is made to halogenide compounds, is there concern with the transport of electric charge through conductive glass, which is coated with a secondary-emissive layer, this being in contradistinction to the tube according to the invention in which the said layer contains sodium- and/or lithium atoms or both. The fact that with this tube such surprising results are obtained could be accounted for by the following theory, which is not, however, to be considered as limiting.

It is presumably ions, emanating from the coating, that transport the charge through the glass. It might be that ions of the monovalent elements sodium and lithium are particularly suitable thereto, since, owing to their small size, they are sufficiently movable in the glass.

The invention may be carried into effect by using as substance for the coating a chlorine compound, such as sodium chloride.

Further development of the invention has shown that particularly fluorine may be selected as the halogen and that cryolite (sodium-aluminum fluoride) is to be considered as an extremely favourable substance for the coating.

In accordance with a further aspect of the invention, atoms of a trivalent, fluorine-binding metal are applied to the coating containing a fluoride compound, the quantity of this metal being such that the surface conductivity and the secondary-emission coefficient of the coating are substantially not affected and that the majority of the fluorine atoms added initially to the sodium or lithium atoms in the coating are bound. It is thus ensured that during the operation of the tube free fluorine atoms produced by secondary emission of the coating are bound with certainty in the coating, so that they do not emerge from the coating and wander through the tube. Trivalent metals suitable to this end are, for example, antimony, bismuth, indium and arsenic. Use is preferably made of antimony. The atoms of this metal form, on the coating, a compound with the available cesium atoms, so that a compound having a comparatively low electrical conductivity is obtained. Even in the case of a comparatively large quantity of antimony on the coating the surface resistance thereof is little affected. A further advantage of antimony is that it hinders little the movement of the primary and secondary electrons striking the coating.

The invention will be described more fully with reference to the drawing, which shows diagrammatically one embodiment of a camera tube according to the invention in a sectional view and the principal electrical connections.

Referring to the drawing, reference numeral 1 designates an exhausted glass vessel, consisting of two cylindrical parts of different diameters and one side tube.

The part having the larger diameter is closed by a glass bottom 2, in which the support 3 for a metal supporting plate 4 for the image electrode 5 is secured. The support 3 establishes the electrical connection with the supporting plate. On the image electrode 5 is applied, for example, a cryolite coating 15 to enhance the secondary emission of the image electrode.

The part having the smaller diameter is closed by a flat glass bottom 6, to the inner side of which is applied

the photo-electric cathode 7. The cathode may, as usual, be made of antimony activated by cesium. Reference numeral 8 designates an optical system, by means of which a luminous image can be projected onto the photo-electric cathode.

To the coating 15 is applied by vaporisation a small quantity of antimony. The antimony may be applied directly after or, if desired, partly simultaneously with the application by vaporisation of the cryolite of the coating 15. The quantity of antimony applied is about 1% by weight of the applied quantity of cryolite in the coating 15. This quantity of antimony does not introduce an appreciable change of the electrical surface resistance of the coating 15, so that the image sharpness is not affected. The secondary-emission coefficient of the coating appears to be slightly higher owing to the antimony; this is believed to be due to a reduction in emission potential, owing to the formation of an antimony-cesium compound on the surface of the coating 15, the cesium, of course, originating from the photo-cathode 7.

In the side tube 9 is arranged an electrode system 10, which serves to produce an electron beam of definite intensity. The axis of this system is directed to the centre of the image electrode 5. By means of the conventional deflection coils 11 and 12 the path of the electron beam can be controlled and by suitable energization of the coils 11 and 12 the complete image surface of the image electrode is periodically scanned by the electron beam.

The wall of the tube has a conductive coating 13, which is electrically connected to an annular collector 14, arranged in the proximity of the image electrode.

The image electrode 5 is formed by a conductive glass layer of about  $60\mu$  applied to the metal supporting plate 4. The specific resistance of this glass is about  $10^{11}$  ohm-cm. under the conditions of operation of the tube. On the image side the conductive glass is coated with a layer of cryolite 15 of about 500 Å. in thickness, precipitated from the vapour phase.

On the wall inside the side tube 9 provision is made of an annular gold layer 16. This layer serves as a store for, or supply of, cesium, but provides at the same time that no excess of cesium vapour is contained in the tube, which would be harmful to the sensitivity of the photo-electric cathode. The cesium is adsorbed by the gold layer when cesium vapour is introduced into the tube during manufacture. The gold layer keeps the cesium away from the electrode system 10.

The current conductor 3 is connected through a load resistor 17 to the negative terminal of a direct-current source 18, the positive terminal of which is connected to the coating 13 and hence also to the collector 14, so that the latter will attract electrons produced by the image electrode 5. A second direct-current source 19 supplies the voltage to produce the scanning beam and serves, moreover, to provide a suitable negative potential at the photo-electric cathode 7 with respect to the coating 13 and the collector 14. The potential difference between the collector and the electrode system 10 with the photo-electric cathode is high with respect to the difference between the collector and the supporting plate 4, so that both the electrons of the scanning beam and the electrons emanating from the photo-electric cathode strike the cryolite layer 15 with a sufficient velocity to set free secondary electrons from this layer.

When struck by the scanning beam, each point of the surface of the image electrode is brought to a potential which is approximately equal to that of the collector. During the time interval between two successive scanings (frame period) the potential of the point is reduced since the image electrode is traversed by electric charge. Owing to this potential drop secondary electrons set free by the photo-electrons during the frame period can be attracted and collected by the collector 14. Conse-

quently, this is only possible when the image electrode has a certain amount of conductivity.

The secondary-emission coefficient of the cryolite layer 15 is particularly high. Values between 9 and 11 are found. These high values are also ascribed to the presence of cesium in the tube. Cesium adheres readily to antimony and halogenide ions, particularly to those of fluorine, which substance is contained in the cryolite. For a large part the favourable properties of the tube according to the invention may be due to these conditions.

It is assumed that cesium atoms adsorbed at the surface of the coating could then bind halogenide atoms, while forming ions, these halogenide atoms being produced when halogenide ions give off electrons by secondary emission. This bond could prevent the halogenide atoms from leaving the coating and from spreading in the tube, and from affecting the photo-electric cathode.

Consequently, the tube should contain cesium. In the embodiment described this substance is provided in the photo-electric cathode. If this is not the case, a separate supply of cesium can be provided. This provision may, otherwise, also be made when the photo-electric cathode already contains cesium, since experiments have shown that an excessively small supply of cesium in the tube may imply that after some time such a quantity of cesium may be withdrawn from the photo-cathode that the effect of this cathode falls off. In the embodiment described a cesium supply is formed by the gold layer 16 in the side tube 9.

When the coating of the tube according to the invention contains fluorine, as is the case with the example described, the spreading of fluorine atoms affecting the photo-electric cathode in the tube is avoided with certainty by applying to the coating by vaporisation a small quantity of atoms of a trivalent, fluorine-binding metal. Such a metal may, for example, be antimony, bismuth, indium or arsenic; use is preferably made of antimony, as is indicated above in the description of the example.

Camera tubes for television exhibit rather often a troublesome phenomenon, referred to as "inscription." This phenomenon consists in that during the use of the tube the coefficient of the secondary emission is changed at those areas of the image electrode which have been loaded most. This drawback may sometimes be obviated or at least reduced by taking the tube out of operation for some time.

Cryolite has the favourable property that it does not or substantially not exhibit the aforesaid phenomenon of "inscription." Since it is, moreover, readily precipitated from the vapour phase in the tube itself on the conductive glass, it is an excellent material for the manufacture of the secondary-emissive coating.

What is claimed is:

1. A television camera tube comprising an envelope and inside said envelope the combination comprising a photo-electric cathode and image electrode cooperating to establish a charge pattern on said image electrode corresponding to a televised object, said image electrode including a conductive glass member and a thin, secondary-electron-emissive coating thereon comprising essentially an inorganic halogen compound containing an alkali metal selected from the group consisting of sodium and lithium, said tube also containing cesium.

2. A television camera tube as set forth in claim 1 wherein the halogen compound is a fluorine compound.

3. A television camera tube as set forth in claim 2 wherein the emissive coating consists essentially of sodium-aluminum fluoride.

4. A television camera tube comprising an envelope and inside said envelope the combination comprising a photo-electric cathode containing cesium and an image electrode cooperating to establish a charge pattern on said image electrode corresponding to a televised object; said image electrode including a glass member having

75 a resistivity within the range from  $10^9$  to  $10^{12}$  ohm-cm.,

an electrode on one side of said glass member, and a thin, secondary-electron-emissive coating on the other side of said glass member and constituted of an inorganic halogen compound containing an alkali metal selected from the group consisting of sodium and lithium; a supply of cesium within said envelope and spaced from said photo-electric cathode; and means for scanning said other side of the image electrode with an electron beam.

5. A camera tube as claimed in claim 2 wherein the emissive coating contains on a surface atoms of a trivalent, fluorine-binding metal in an amount such that the surface conductivity and the secondary-emission coefficient of the coating are substantially not affected.

6. A camera tube as claimed in claim 5 in which the trivalent metal is antimony.

7. A television camera tube comprising a photo-elec-

tric cathode containing cesium and an image electrode, said image electrode being constituted of a glass member having a resistivity in the range of  $10^9$  to  $10^{12}$  ohm-cm., and a thin cryolite coating on said glass member.

8. A tube as set forth in claim 7 wherein antimony is present on the cryolite coating.

9. A tube as set forth in claim 8 wherein the antimony constitutes about 1% by weight of the cryolite, and the cryolite coating has a thickness of about 500 Å.

References Cited in the file of this patent

UNITED STATES PATENTS

2,535,817 Skellett \_\_\_\_\_ Dec. 26, 1950  
2,547,638 Gardner \_\_\_\_\_ Apr. 3, 1951

FOREIGN PATENTS

510,784 Canada \_\_\_\_\_ Mar. 8, 1955